

## UNITED STATES PATENT OFFICE

1,957,020

## PROCESS FOR TREATING HIDES

Herbert C. Reed, Stamford, Conn., assignor to  
 Niacet Chemicals Corporation, a corporation  
 of New York

No Drawing. Application August 5, 1931,  
 Serial No. 555,370

13 Claims. (Cl. 149—5)

The invention relates to a process for treating hides as an aid in the production of leather.

Hides are usually received at the tannery after they have been cured by salting or sun-drying. At the tannery they are cleansed and rehydrated by soaking and washing the hides in water. They are then unhaired, plumped, and finally tanned, whereby the tissues of the hides are converted into tough, imputrescible substances. In some instances the hides may be subjected to a bathing process wherein the hides are depleted and softened by the putrefactive or fermentive action of a bacteriological bath.

It is not always practical or feasible to conduct the treatment of the hides at the tannery in an uninterrupted sequence of operations. For this reason difficulties are encountered and losses occur due to the excessive putrefaction of hides which are allowed to stand between the various steps in their treatment. This spoilage is particularly prevalent in hides which have been bated and which are not immediately processed further. Also, hides which are cured by salting are frequently unfit for the production of certain types of leather. For example, goat or kid skins from which white or light-colored leather is to be prepared may exhibit dark stains when tanned due to the presence of iron impurities in the salt with which the hides are cured. These iron compounds, if not entirely removed by repeated and protracted washings, are precipitated by the tanning agent and produce the objectionable stains.

These difficulties are largely avoided and novel benefits are derived from the application of the process of the present invention to the treatment of hides. The invention comprises, as its principal feature of novelty, the application of treating agents not heretofore used for this purpose, and provides a simple, efficient and economical method for treating hides preliminary to tanning, all as more fully hereinafter described.

In practicing my invention, the hides, prior to or at the beginning of the tanning operations, are subjected to the action of an aqueous solution of 45 paraldehyde (paracetaldehyde,  $(\text{CH}_3\text{CHO})_2$ ), or paraldol ( $\text{CH}_3\text{CHOH.CH}_2\text{CHO}$ ).

This treatment preferably occurs at the tannery, but, in the case of paraldehyde, may occur immediately after flaying to replace other curing methods. In general, the hides are soaked with or without agitation in a bath containing from about 0.1% to 10% of either paraldehyde or paraldol based on the weight of the hides. Lower concentrations of the treating agent in the bath 55 within the range indicated, and shorter immerge-

sion times may be used if the bath is thoroughly agitated.

The effect of this treatment is multi-fold; it cleanses the hides, preserves the hides, plumps and fulls them, and, at least in the case of 63 paraldehyde, exerts a beneficial preservative effect upon certain vegetable tanning agents with which the hides may be subsequently contacted.

The application of the two treating agents of my invention follow each other in nearly all respects. The principal difference is in regard to their use in conjunction with lime baths or lime depilatory treatments. Paraldol cannot be advantageously used simultaneously with such treatments because the paraldol tends to react 73 with lime. For this reason treatment with paraldol should be carried out after the hides have received the lime treatment, or treatment with other strongly alkaline materials.

The treatment with paraldehyde may occur at 75 any time before tanning whether it is before, after or during lime treatment.

The following examples are illustrative of the invention:

I. One hundred pounds of wet goatskins were 80 placed in a drum containing 3 pounds of paraldehyde and 97 pounds of water. The skins were thoroughly agitated in this bath for one hour and were then removed, allowed to drain, and were introduced directly into the tanning bath.

II. The process of Example I was varied by 85 using 5 pounds of paraldehyde and 95 pounds of water, and 30 minutes of agitation in the bath. The cleansing and plumping effects secured in each case were very similar.

Hides which have been subjected to a bathing treatment may be immediately thereafter treated with paraldehyde in the manner described. This treatment cleanses and plumps the hides, and in addition, it prevents putrefaction, allowing the 95 hides to be transported or stored for considerable periods of time without spoilage.

Hides or skins which have been treated with paraldehyde or paraldol yield a higher grade of leather than similar hides which are tanned in 100 the same manner without the use of these agents. The treatment of my invention plumps and fulls the hide, giving it a rubbery feel, and causing it to become slippery on both the flesh and grain sides. The hides, after being treated with the 105 new treating agents, may be removed from the bath and then tanned or the tanning may be accomplished by adding a tanning agent to the treating solution thus avoiding the necessity of transferring the hides to another bath.

110

From the foregoing description it will be apparent that modifications of my new process are possible and are included within the scope of the invention as defined by the appended claims.

5 I claim:

1. A process for treating hides preliminary to tanning operations which comprises soaking the hides in a bath containing a substance of the group consisting of paraldehyde and paraldol. 80
- 10 2. A process for treating hides preliminary to tanning operations which comprises soaking the hides in a bath containing about 0.1% to 10% based on the wet weight of the hides, of a substance of the group consisting of paraldehyde and 85 paraldol. 90
- 15 3. A process for treating hides to obtain leather therefrom which includes the steps of soaking the hides in a bath containing paraldehyde, drying the skins, rehydrating the hides and finally 20 tanning the hides. 95
- 20 4. A process for treating hides to obtain leather therefrom which includes the steps of soaking the hides in a bath containing about 0.1% to 10% of paraldehyde based on the wet weight of the 25 hides. 100
- 25 5. A process for treating hides to obtain leather therefrom which includes the steps of soaking the hides in a bath containing paraldehyde until the hides are plumped, and then adding a tanning 30 agent to said bath to convert the tissues of said hides into tough, imputrescible substances. 105
- 30 6. A process for treating hides to obtain leather therefrom which includes the steps of soaking the hides in a bath containing about 0.1% to 10% of paraldehyde based on the wet weight of the 35 hides until the hides are plumped, and then adding a tanning agent to said bath to convert the tissues of said hides into tough, imputrescible 110 substances. 115
- 40 7. A process for treating hides preliminary to HERBERT C. REED. 115

45

120

50

125

55

130

60

135

65

140

70

145

75

150

tanning operations which comprises agitating the hides in an aqueous bath containing about 3% of paraldehyde, based on the wet weight of the hides until the hides are plumped and swelled. 80

8. A process for treating hides preliminary to tanning operations which comprises agitating the hides for about one hour in an aqueous bath containing about 3% of paraldehyde, based on the wet weight of the hides. 85

9. A process for treating hides to obtain leather therefrom which includes the steps of soaking the hides in a bath containing about 0.1% to 10% of paraldol based on the wet weight of the hides. 90

10. A process for treating hides to obtain leather therefrom which includes the steps of soaking the hides in a bath containing paraldol until the hides are plumped, and then adding a tanning agent to said bath to convert the tissues of said hides into tough, imputrescible substances. 95

11. A process for treating hides to obtain leather therefrom which includes the steps of soaking the hides in a bath containing about 0.1% to 10% of paraldol based on the wet weight of the hides until the hides are plumped, and then adding a tanning agent to said bath to convert the tissues of said hides into tough, imputrescible substances. 100

12. A process for treating hides preliminary to tanning operations which comprises agitating the hides in an aqueous bath containing about 3% of paraldol, based on the wet weight of the hides until the hides are plumped and swelled. 105

13. A process for treating hides preliminary to tanning operations which comprises agitating the hides for about one hour in an aqueous bath containing about 3% of paraldol, based on the wet weight of the hides. 110